

Dec. 22, 1931.

A. HELLERMANN

1,838,064

RAILWAY OR TRAMWAY RAIL JOINT

Filed Aug. 10, 1929



August Hellermann.

Inventor,  
Ernst J. Michaelis  
Attorney.

## UNITED STATES PATENT OFFICE

AUGUST HELLERMANN, OF DUSSELDORF-OBERKASSEL, GERMANY, ASSIGNOR TO THE FIRM GESELLSCHAFT FUR WIRTSCHAFTLICHEN BAHNOBERBAU M. B. H., OF FREIBURG, GERMANY

## RAILWAY OR TRAMWAY RAIL JOINT

Application filed August 10, 1929, Serial No. 384,880, and in Germany April 4, 1927.

My invention relates to railway or tramway rail joints in which the abutting ends of the rails are connected by means of fish plates welded to the rails, and has for an object to provide an improved construction such that rupture of the weld is avoided and liability to injury to the rails by the wheel load in the neighbourhood of the joint is obviated.

In previously known rail joints of this kind considerable internal strains are set up in the welded seams in consequence of the contraction on cooling, as a result of which and of the stresses occasioned on the passage of vehicles over the rails the weld is liable to give way prematurely.

It has been ascertained as the result of experimental research that the shrinkage of the weld diminishes the rail height by about

1.5 millimetres if no resistance is offered by the rail web. This reduction in height is equivalent to an expansion strain of about 5%. Besides these internal strains the weld is subject to other stresses due to the altered static condition of the rails in the vicinity of the joint. The fish plate connection which functions as a rigid connection in consequence of the welding opposes the depression curve or deflection wave which accompanies the

travel of the wheel over the rail. Whereas away from the joint the rail is loaded after the fashion of a beam freely supported at both ends, shortly in front of the fish plate connection there is an extra load which cor-

responds to the loading of a beam at one side. The compression stresses which are set up in the rail heads in consequence of the deflection are accordingly converted into tensile stresses in front and beyond the butt joint.

The change of load which takes place in a very brief time is a cause of breakage of the rails or injury thereto shortly in front of the fish-plate joint. Besides these static strains of the seams and of the rails there are

set up powerful stresses in the neighbourhood of the joints due to the dynamic action between the rail and the wheel. Due to the altered static relation there is in the neighbourhood of the butt joint a sudden alteration of the deflection

wave which accompanies the rolling wheel and therefore a sudden alteration in the direction of movement of the wheel. A further unfavourable factor is that with the heretofore usual construction of the parts forming the joint there is a local accumulation of material so that the natural deflection wave is opposed by the substantial inertia at this point. The stresses consequent on sudden change of direction of the wheel may therefore prove destructive to the joint.

Starting from the recognition of these phenomena, according to my present invention I make provision whereby the setting up of internal strains in the seams in consequence of contraction and also local accumulation of material and alteration in the static conditions in the neighbourhood of the joint are obviated.

According to my invention, the parts in the neighbourhood of the joint that are to be welded together are made yielding by longitudinal interruptions in the direction of the forces set up on contraction of the seams so that they can follow the movement of contraction without occasioning internal strains.

In the accompanying drawings which illustrate the invention Figs. 1 and 2 show in side elevation and in section on the line 2—2 of Fig. 1, respectively, a rail joint with short fish-plates of rectangular form welded to the rail ends.

Figs. 3 and 4 show in side elevation and in section on the line 4—4 of Fig. 3, respectively, a rail joint in which the fish-plates are made yielding in vertical direction by the provision of wedge-shaped notches which extend up to the short middle portion.

Figs. 5 to 7 show a rail joint with bridge-pieces arranged superposed on the welded fish-plates, Fig. 5 being a side elevation, Fig. 6 a section on the line 6—6, and Fig. 7 a section on the line 7—7 of Fig. 5.

Figs. 8 and 9 show in side elevation and in section on the line 9—9 of Fig. 8 a modified construction incorporating half fish-plates adjustable in the direction of the forces set up on contraction.

Figs. 10 and 11 show in side elevation and

in section on the line 11—11 of Fig. 10, respectively, a further modification.

Referring to Figs. 1 to 7 of the drawings, the webs *a*, *b* of the abutting rail ends *a*, *b* are formed with slots *c*, *d* in the neutral zone of the rails, so that the heads and bases of the rail ends can follow the contractile movement of the welded seams *e*, *f* which serve in known manner to connect the fish-plates *g* with the rail ends. After the fish-plates *g* have been welded to the rail ends, the slots *c*, *d* are filled with weld metal on both sides of the fish-plates. By the contraction of the weld metal filling the slots there are set up in the seams *e* and *f* compression strains which oppose the tensile strains in the seams when a wheel travels over the joint. To prevent excessive rigidity which would unfavourably affect the static condition of the rails in the neighbourhood of the joint, in the construction shown in Figs. 1 and 2 the welded fish-plates *g* and thus also the seams *e* and *f* are short. This construction, however, is recommended only in the case where the forces acting in the longitudinal direction of the rails are small. In order to avoid exposing the seams *e* and *f* to transverse stresses on the passage of a wheel over the joint, the fish-plates *e* are pressed by means of bolts *i* against the bases and heads of the rail ends.

In the construction shown in Figs. 3 and 4 the fish-plates *g* and the seams *e* and *f* are relatively long. In order to ensure that the rails may yield sufficiently in the neighbourhood of the joint, the fish-plates are each formed at their ends with wedge-shaped notches *h* of such length that there is left only a relatively small middle portion *g'* which is rigid in vertical direction. The notches *h* are so arranged that the slots *c* and *d* in the webs can be filled with weld metal up to the rigid middle portions of the fish-plates. As in the construction shown in Figs. 1 and 2 the fish-plates are held pressed against the heads and bases of the rail ends by means of a bolt *i*.

In the construction shown in Figs. 5 to 7 there are superposed on the fish-plates *g* bridge-pieces *h* serving to transmit the forces acting in the longitudinal direction of the rails. To provide a joint rigid in longitudinal direction between the bridge-pieces and the rail ends *a* and *b* there are provided two sleeves *l* fitted to the ends of the bridge-pieces and each having an eccentric central portion *l'* fitted in a cylindrical enlargement of the slot *c* or *d*, so that by turning the sleeves about their axes variation in spacing of the apertures in the bridge piece to be traversed by the sleeves may be accommodated. To ensure that the rigidity of the joint in vertical direction will not be materially increased by the provision of such bridge-pieces the latter are so held to the sleeves *l*

by means of bolts *m* penetrating the sleeves that, on deflection of the rail ends under the action of the wheel load the bridge-pieces can turn about the sleeves. The bridge-pieces *h* are held pressed against the welded fish-plates at their centres by means of a bolt *n* so that they take up the transverse stresses exercised on the fish-plates when a vehicle wheel passes over the joint. In order that this bolt may not prevent the rocking movement of the bridge-pieces *h* around the sleeves *l* play is allowed between the bolt on the one hand, and the rail web, the fish-plates and the bridge-pieces on the other hand. Also, in this construction, the slots *c* and *d* are filled with weld metal up to the fish-plates *g*. As the sleeves *l* are mounted in cylindrical enlargements of the slots *c* and *d*, they are locked against movement after the closure of the slots by weld metal in consequence of the contraction of the seams.

In the construction shown in Figs. 8 and 9 each of the fish-plates welded to the rails consists of two sections *o* and *p*. The adjacent edges of these half fish-plates *o* and *p* are inclined in longitudinal direction and co-operate with relatively adjustable wedges *q* and *r* in such wise that the half fish-plates *o* and *p* can follow the contractile movements of the seams *e* and *f* on cooling.

The wedges are connected by a horizontal bolt *s* on which is threaded a nut *t* by adjustment of which the spacing of the wedges *q* and *r* can be varied, so that the half fish-plates *o* and *p* may be urged apart and the seams *e* and *f* subjected to compression. The wedges *r* are each provided with a longitudinal slot *u* penetrated by a bolt *v* serving to take up transverse stresses. Between the half fish-plates *o* and *p* and the heads on the one hand and bases of the rail ends on the other hand are interposed strips *e'* and *f'* of yielding heat-resisting material, for example, mica, in order to permit the half fish-plates to yield relatively to the heads and bases of the rail ends on contraction of the seams and to smooth out unevenness of the abutting surfaces. To prevent transverse shift of the wedges *q* and *r* relatively to the half fish-plates *o* and *p*, the wedges are provided with longitudinal grooves entered by the edges of the half fish-plates.

In the construction shown in Figs. 10 and 11 the half fish-plates *o* and *p* are engaged by two clamping jaws *w* and *x*, penetrating the rail webs. These jaws are guided in notches *w'*, *x'* in the rail webs so that they are movable in vertical direction only. Near the ends of the jaws are grooves *w<sup>2</sup>*, *x<sup>2</sup>* engaged by the half fish-plates *o*, *p*. To urge apart the jaws *w* and *x* there are driven between the same two wedges *y*, *z* of which the wedge *y* extends over the entire length of the jaws while the wedge *z* is of

such length that in conjunction with the thick end of the wedge  $y$  it acts on half only of the jaws. The wedge  $y$  has upset portions  $y'$   $y^2$  at both ends of which one portion  $y'$  bears against the face of the jaw  $x$  while the other portion  $y^2$  engages the thick end of the wedge  $z$ . The wedges are thus held against working loose. The upset portions  $y$  and  $y^2$  are narrower than the wedge proper  $y$  so that they do not hinder the driving of the wedge. With this formation and arrangement of the jaws the use of bolts etc. for spacing the half fish-plates and for pressing the same against the rail ends may be dispensed with. Depending on the length of the fish-plates there may be provided several such clamping devices acting on the ends of the half fish-plates, this last mentioned arrangement being particularly applicable to low rails in which the available space is insufficient to accommodate clamping means at the centre, that is, at the point where the fish-plates are subject to maximum stresses.

25 In the construction shown in Figs. 10 and 11 slotting of the rail webs is unnecessary. If desired, however, the rail webs may be slotted in the constructions shown in Figs. 8 and 9 and in Figs. 10 and 11. 30 For example, it is possible by means of such slots to accommodate unevenness at the joints. Further, these slots may be filled with weld metal as in the other constructions described.

35 What I claim as my invention and desire to secure by Letters Patent of the United States, is:

1. A rail joint, comprising, in combination, two abutting rail ends, fish-plates welded to the heads and bases of said rail ends, and longitudinal interruptions in one of said parts united by welding, said interruptions being disposed so that said parts united by welding are free to follow the movements produced by forces set up on contraction of the welding seams, whereby the production of internal strains in the parts welded is obviated.

2. A rail joint, comprising, in combination, two abutting rail ends, fish-plates welded to the heads and bases of said rail ends, and slots in the webs of said rail ends, said slots being disposed in the neutral zone of said webs, whereby the heads and bases of said rail ends are free to follow the movements produced by forces set up on contraction of the welding seams.

3. A rail joint, comprising, in combination, two abutting rail ends, a fish-plate welded to the heads and bases of said rail ends, and longitudinal interruptions in one of said parts united by welding, said interruptions being disposed so that said parts united by welding are free to follow the movements produced by forces set up on contraction of the welding

ing seams, whereby the production of internal strains in the parts welded is obviated, said interruptions being filled with weld metal after said fish-plate has been welded to said rails.

4. A rail joint, comprising, in combination, two abutting rail ends, a fish-plate welded to the heads and bases of said rail ends, and slots in the neutral zone of the webs of said rail ends, whereby the heads and bases of said rail ends united by welding are free to follow the movements produced by forces set up on contraction of weld seams, said slots being filled with weld metal at both sides of said fish-plate after the latter has been united to said rails.

5. A rail joint, comprising, in combination, two abutting rail ends, a fish-plate welded to the heads and bases of said rail ends, and longitudinal interruptions in one of said parts united by welding, said interruptions being disposed so that said parts united by welding are free to follow the movements produced by forces set up on contraction of the seams, whereby the production of internal strains in the parts welded is obviated, said fish-plates being provided with preferably wedge-shaped notches extending from the ends of said fish-plate and of such length that said fish-plate is yielding in vertical direction save for a relatively small middle portion.

6. A rail joint, comprising, in combination, two abutting rail ends, and a fish-plate welded to the heads and bases of said rail ends, said fish-plate being provided with preferably wedge-shaped notches extending from the ends of said fish-plate and of such length that said fish-plate is yielding in vertical direction save for a relatively small middle portion.

7. A rail joint, comprising, in combination, two abutting rail ends, a fish-plate welded to the heads and bases of said rail ends, and slots in the neutral zone of the webs of said ends, whereby the heads and bases of said rail ends united by welding are free to follow the movements produced by forces set up on contraction of the weld seams, said fish-plate being provided with preferably wedge-shaped notches extending from the ends of said fish-plate and of such length that said fish-plate is yielding in vertical direction save for a relatively small middle portion, said slots being filled with weld metal at both sides of said fish-plate after the latter has been united to said rails.

8. A rail joint, comprising, in combination, two abutting rail ends, a fish-plate welded to the heads and bases of said rail ends, longitudinal interruptions in one of said parts united by welding, said interruptions being disposed so that said parts united by welding are free to follow the movements produced by forces set up on contraction of the welding

- seams, whereby the production of internal strains in the parts welded is obviated, and a bridge-member arranged in front of said fish-plate and so connected with said rail ends that said bridge-member transmits the forces acting in the longitudinal direction of said rails while relieving the seams.
9. A rail joint, comprising, in combination, two abutting rail ends, fish-plates welded to the heads and bases of said rail ends, slots in the webs of said rail ends, said slots being disposed in the neutral zone of said webs, whereby the heads and bases of said rail ends are free to follow the movements produced by forces set up on contraction of the welding seams, and a bridge-member arranged in front of said fish-plates and so connected with said rail ends that said bridge-member transmits the forces acting in the longitudinal directions of said rails while relieving the seams.
10. A rail joint, comprising, in combination, two abutting rail ends, a fish-plate welded to the heads and bases of said rail ends, longitudinal interruptions in one of said parts united by welding, said interruptions being disposed so that said parts united by welding are free to follow the movements produced by forces set up on contraction of the welding seams, whereby the production of internal strains in the parts welded is obviated, said interruptions being filled with weld metal after said fish-plate has been welded to said rails, and a bridge-member arranged in front of said fish-plate and so connected with said rail ends that said bridge-member transmits the forces acting in the longitudinal directions of said rails while relieving the seams.
11. A rail joint, comprising, in combination, two abutting rail ends, a fish-plate welded to the heads and bases of said rail ends, slots in the neutral zone of the webs of said rail ends, whereby the heads and bases of said rail ends united by welding are free to follow the movements produced by forces set up on contraction of weld seams, said slots being filled with weld metal at both sides of said fish-plate after the latter has been united to said rails, and a bridge-member arranged in front of said fish-plate and so connected with said rail ends that said bridge-member transmits the forces acting in the longitudinal directions of said rails while relieving the seams.
12. A rail joint, comprising, in combination, two abutting rail ends, a fish-plate welded to the heads and bases of said rail ends, and longitudinal interruptions in one of said parts united by welding, said interruptions being disposed so that said parts united by welding are free to follow the movements produced by forces set up on contraction of the seams, whereby the production of internal strains in the parts welded is

- obviated, said fish-plate being provided with preferably wedge-shaped notches extending from the ends of said fish-plate and of such length that said fish-plate is yielding in vertical direction save for a relatively small middle portion, and a bridge-member arranged in front of said fish-plate and so connected with said rail ends that said bridge-member transmits the forces acting in the longitudinal directions of said rails while relieving the seams.
13. A rail joint, comprising, in combination, two abutting rail ends, a fish-plate welded to the heads and bases of said rail ends, said fish-plate being provided with preferably wedge-shaped notches extending from the ends of said fish-plate and of such length that said fish-plate is yielding in vertical direction save for a relatively small middle portion, and a bridge-member arranged in front of said fish-plate and so connected with said rail ends that said bridge-member transmits the forces acting in the longitudinal directions of said rails while relieving the seams.
14. A rail joint, comprising, in combination, two abutting rail ends, fish-plates welded to the heads and bases of said rail ends, longitudinal interruptions in one of said parts united by welding, said interruptions being disposed so that said parts united by welding are free to follow the movements produced by forces set up on contraction of the welding seams, whereby the production of internal strains in the parts welded is obviated, a bridge-piece arranged in front of each fish-plate, and a pivotal connection between each end of said bridge-piece and the adjoining rail web, whereby said bridge-piece is adapted to simultaneously transmit forces acting in longitudinal direction of said rails and to rock in vertical direction.
15. A rail joint, comprising, in combination, two abutting rail ends, fish-plates welded to the heads and bases of said rail ends, slots in the webs of said rail ends, said slots being disposed in the neutral zone of said webs, whereby the heads and bases of said rail ends are free to follow the movements produced by forces set up on contraction of the welding seams, a bridge-piece arranged in front of each fish-plate, and a pivotal connection between each end of said bridge-piece and the adjoining rail web, whereby said bridge-piece is adapted to simultaneously transmit forces acting in longitudinal direction of said rails and to rock in vertical direction.
16. A rail joint, comprising, in combination, two abutting rail ends, a fish-plate welded to the heads and bases of said rail ends, slots in the neutral zone of the webs of said rail ends, whereby the heads and bases of said rail ends united by welding are free to follow the movements produced by forces set

up on contraction of weld seams, said slots being filled with weld metal at both sides of said fish-plate after the latter has been united to said rails, a bridge-piece arranged in front of said fish-plate, and a pivotal connection between each end of said bridge-piece and the adjoining rail web, whereby said bridge-piece is adapted to simultaneously transmit forces acting in longitudinal direction of said rails and to rock in vertical direction.

17. A rail joint, comprising, in combination, two abutting rail ends, a fish-plate welded to the heads and bases of said rail ends, said fish-plate being provided with preferably wedge-shaped notches extending from the ends of said fish-plate and of such length that said fish-plate is yielding in vertical direction save for a relatively small middle portion, and a bridge-piece in front of said fish-plate, and a pivotal connection between each end of said bridge-piece and the adjoining rail web, whereby said bridge-piece is adapted to simultaneously transmit forces acting in longitudinal direction of said rails and to rock in vertical direction.

18. A rail joint, comprising, in combination, two abutting rail ends, fish-plates welded to the heads and bases of said rail ends, slots in the webs of said rail ends, said slots being disposed in the neutral zone of said webs, whereby the heads and bases of said rail ends are free to follow the movements produced by forces set up on contraction of the welding seams, a bridge-piece arranged in front of each fish-plate, and a pivotal connection between each end of said bridge-piece and the adjoining rail web, said pivotal connection comprising an adjustment member adapted to be fixed in its adjusted position by forces set up on contraction of the welding seams.

19. A rail joint, comprising, in combination, two abutting rail ends, a fish-plate welded to the heads and bases of said rail ends, slots in the neutral zone of the webs of said rail ends, whereby the heads and bases of said rail ends united by welding are free to follow the movements produced by forces set up on contraction of weld seams, said slots being filled with weld metal at both sides of said fish-plate after the latter has been united to said rails, a bridge-piece in front of said fish-plate, and a pivotal connection between each end of said bridge-piece and the adjoining rail web, said pivotal connection comprising an adjustment member adapted to be fixed in its adjusted position by forces set up on contraction of the welding seams.

20. A rail joint, comprising, in combination, two abutting rail ends, a fish-plate welded to the heads and bases of said rail ends, said fish-plate being provided with preferably wedge-shaped notches extending from the ends of said fish-plate and of such

length that said fish-plate is yielding in vertical direction save for a relatively small middle portion, a bridge-piece arranged in front of each fish-plate, and a pivotal connection between each end of said bridge-piece and the adjoining rail web, said pivotal connection comprising an adjustment member adapted to be fixed in its adjusted position by forces set up on contraction of the welding seams.

21. A rail joint, comprising, in combination, two abutting rail ends, fish-plates welded to the heads and bases of said rail ends, each fish-plate comprising superposed parts and means for pressing said parts against heads and bases of the respective rail ends.

22. A rail joint, comprising, in combination two abutting rail ends, fish-plates welded to the heads and bases of said rail ends, each fish-plate comprising superposed parts and means for pressing said parts against heads and bases of the respective rail ends, and spacing members of a yielding and heat-resisting character interposed between each rail head and rail base and the respective fish-plate parts pressed against said rail heads and rail bases by said pressing means.

23. A rail joint, comprising, in combination, two abutting rail ends, fish-plates welded to the heads and bases of said rail ends, each fish-plate comprising superposed parts and means for pressing said parts against heads and bases of the respective rail ends, said pressing means comprising wedge members and adjustable means for varying the wedge action of said wedge members, said wedge members and fish-plate parts engaging each other by means of a tongue and groove engagement.

24. A rail joint, comprising, in combination, two abutting rail ends, fish-plates welded to the heads and bases of said rail ends, each fish-plate comprising superposed part and means for pressing said parts against heads and bases of the respective rail ends, said pressing means comprising vertically adjustable clamping jaws and wedges for actuating said clamping jaws, the latter being guided in perforations of the rail webs in such wise that they act simultaneously on said fish-plate parts on both sides of the rail.

25. A rail joint, comprising, in combination, two abutting rail ends, fish-plates welded to the heads and bases of said rail ends, each fish-plate comprising superposed parts and means for pressing said parts against heads and bases of the respective rail ends, said pressing means comprising vertically adjustable clamping jaws and wedges for actuating said clamping jaws, the latter being guided in perforations of the rail webs in such wise that they act simultaneously on said fish-plate parts on both sides of the rail, said actuating wedges consisting of a pair of wedges adapted to co-operate with each pair

of clamping jaws in such wise that the forces exercised on said fish-plate parts at each rail side can be adjusted independently.

26. A rail joint, comprising, in combination, two abutting rail ends, a fish-plate welded to the heads and bases of said rail ends, longitudinal interruptions in one of said parts united by welding, said interruptions being disposed so that said parts united by welding are free to follow the movements produced by forces set up on contraction of the welding seams, whereby the production of internal strains in the parts welded is obviated, and spacing members interposed between each rail head and each rail base and the respective fish-plate parts, said spacing members are of a yielding and heat-resisting character and do not extend into the adjoining weld seams.

27. In testimony whereof I affixed my signature.

AUGUST HELLERMANN.